



US008168358B2

(12) **United States Patent**  
**Wu**

(10) **Patent No.:** **US 8,168,358 B2**  
(45) **Date of Patent:** **\*May 1, 2012**

(54) **POLYSULFONE CONTAINING  
PHOTOCODUCTORS**

(75) Inventor: **Jin Wu**, Webster, NY (US)

(73) Assignee: **Xerox Corporation**, Norwalk, CT (US)

(\*) Notice: Subject to any disclaimer, the term of this patent is extended or adjusted under 35 U.S.C. 154(b) by 446 days.

This patent is subject to a terminal disclaimer.

(21) Appl. No.: **12/493,481**

(22) Filed: **Jun. 29, 2009**

(65) **Prior Publication Data**

US 2010/0330478 A1 Dec. 30, 2010

(51) **Int. Cl.**  
**G03G 5/04** (2006.01)

(52) **U.S. Cl.** ..... **430/58.8**; 430/58.15; 430/59.6

(58) **Field of Classification Search** ..... **430/58.8,**  
430/58.15; 524/167

See application file for complete search history.

(56) **References Cited**

U.S. PATENT DOCUMENTS

4,555,463 A 11/1985 Hor et al.  
4,587,189 A 5/1986 Hor et al.

|                   |         |                              |
|-------------------|---------|------------------------------|
| 5,473,064 A       | 12/1995 | Mayo et al.                  |
| 5,482,811 A       | 1/1996  | Keoshkerian et al.           |
| 5,521,306 A       | 5/1996  | Burt et al.                  |
| 6,174,636 B1 *    | 1/2001  | Fuller et al. .... 430/58.7  |
| 6,913,863 B2      | 7/2005  | Wu et al.                    |
| 7,485,398 B2      | 2/2009  | Wu et al.                    |
| 7,553,593 B2      | 6/2009  | Wu et al.                    |
| 8,029,901 B2 *    | 10/2011 | Wu ..... 428/411.1           |
| 2008/0057426 A1 * | 3/2008  | McGuire et al. .... 430/58.8 |
| 2008/0118853 A1 * | 5/2008  | Bender ..... 430/96          |

OTHER PUBLICATIONS

Jin Wu, U.S. Appl. No. 12/059,573 on Oxadiazole Containing Photoconductors, filed Mar. 31, 2008.

Liang-Bih Lin et al., U.S. Appl. No. 12/059,573 on Benzothiazole Containing Photogenerating Layer, filed Mar. 31, 2008.

Jin Wu et al., U.S. Appl. No. 12/059,555 on Thiuram Tetrasulfide Containing Photogenerating Layer, filed Mar. 31, 2008.

Jin Wu et al., U.S. Appl. No. 12/059,587 on Titanocene Containing Photoconductors, filed Mar. 31, 2008.

Jin Wu et al., U.S. Appl. No. 12/059,663 on Thiadiazole Containing Photoconductors, filed Mar. 31, 2008.

\* cited by examiner

*Primary Examiner* — Christopher Rodee

*Assistant Examiner* — Jonathan Jelsma

(74) *Attorney, Agent, or Firm* — Oliff & Berridge, PLC

(57) **ABSTRACT**

A photoconductor that includes, for example, a supporting substrate, a photogenerating layer, and a charge transport layer, and wherein the charge transport layer contains a polysulfone.

**28 Claims, No Drawings**

## 1

POLYSULFONE CONTAINING  
PHOTOCOCONDUCTORSCROSS REFERENCE TO RELATED  
APPLICATIONS

U.S. application Ser. No. 12/059,573, now U.S. Pat. No. 7,960,080, filed Mar. 31, 2008, the disclosure of which is totally incorporated herein by reference, there is illustrated a photoconductor comprising a supporting substrate, a photogenerating layer, and at least one charge transport layer wherein at least one of the charge transport layers is comprised of at least one charge transport component, and wherein at least one of the photogenerating layer, and the charge transport layer includes an oxadiazole.

U.S. application Ser. No. 12/059,478, now U.S. Pat. No. 7,935,466, filed Mar. 31, 2008, the disclosure of which is totally incorporated herein by reference, illustrates a photoconductor comprising a supporting substrate, a photogenerating layer, and a charge transport layer comprised of at least one charge transport component, and wherein the photogenerating layer contains a benzothiazolesulfenimide additive.

U.S. application Ser. No. 12/059,555, now U.S. Pat. No. 7,989,129, filed Mar. 31, 2008, the disclosure of which is totally incorporated herein by reference, illustrates a photoconductor comprising a supporting substrate, a photogenerating layer, and at least one charge transport layer comprised of at least one charge transport component, and wherein the photogenerating layer contains a hydroxyquinoline.

U.S. application Ser. No. 12/059,587, now U.S. Pat. No. 7,811,732, filed Mar. 31, 2008, the disclosure of which is totally incorporated herein by reference, illustrates a photoconductor comprising a supporting substrate, a photogenerating layer, and at least one charge transport layer wherein at least one of the charge transport layers is comprised of at least one charge transport component, and wherein at least one of the photogenerating layer and the charge transport layer includes a titanocene.

U.S. application Ser. No. 12/059,663, now U.S. Pat. No. 7,981,579, filed Mar. 31, 2008, the disclosure of which is totally incorporated herein by reference, illustrates a photoconductor comprising a supporting substrate, a photogenerating layer, and at least one charge transport layer comprised of at least one charge transport component, and wherein the photogenerating layer includes a thiadiazole.

In U.S. application Ser. No. 11/472,765, now U.S. Pat. No. 7,553,593, and U.S. application Ser. No. 11/472,766, now U.S. Pat. No. 7,485,398, the disclosures of which are totally incorporated herein by reference, there are disclosed, for example, photoconductors comprising a photogenerating layer and a charge transport layer, and wherein the photogenerating layer contains a titanyl phthalocyanine prepared by dissolving a Type I titanyl phthalocyanine in a solution comprising a trihaloacetic acid and an alkylene halide; adding the mixture comprising the dissolved Type I titanyl phthalocyanine to a solution comprising an alcohol and an alkylene halide thereby precipitating a Type Y titanyl phthalocyanine; and treating the Type Y titanyl phthalocyanine with a monochlorobenzene.

High photosensitivity titanyl phthalocyanines are illustrated in U.S. application Ser. No. 10/992,500, U.S. Publication No. 20060105254, now U.S. Pat. No. 7,947,417, the disclosure of which are totally incorporated herein by reference, which, for example, discloses a process for the preparation of a Type V titanyl phthalocyanine, comprising providing a Type I titanyl phthalocyanine; dissolving the Type I titanyl phthalocyanine in a solution comprising a trihaloace-

## 2

tic acid and an alkylene halide like methylene chloride; adding the resulting mixture comprising the dissolved Type I titanyl phthalocyanine to a solution comprising an alcohol and an alkylene halide thereby precipitating a Type Y titanyl phthalocyanine; and treating the Type Y titanyl phthalocyanine with monochlorobenzene to yield a Type V Many) phthalocyanine.

A number of the components and amounts thereof of the above copending applications, such as the supporting substrates, resin binders, photogenerating layer components, such as hydroxygallium phthalocyanines, titanyl phthalocyanines, antioxidants, charge transport components, hole blocking layer components, adhesive layers, and the like, may be selected for the members of the present disclosure in embodiments thereof.

## BACKGROUND

This disclosure is generally directed to members like xerographic imaging members, photoreceptors, photoconductors, and the like. More specifically, the present disclosure is directed to rigid, multilayered flexible, belt imaging members, or devices comprised of an optional supporting medium like a substrate, a polysulfone, and more specifically, photogenerating layer, and a polysulfone charge transport layer including a plurality of charge transport layers, such as a first charge transport layer and a second charge transport layer, an optional adhesive layer, an optional hole blocking or undercoat layer, and an optional overcoating layer. At least one in embodiments refers, for example, to one, to from 1 to about 10, to from 2 to about 7; to from 2 to about 4, 1, 2, or 3, 1 or 2, to two, and the like. Moreover, the polysulfone can be added to the charge transport layer instead of being dissolved in the charge transport layer solution.

Yet more specifically, there is disclosed a photoconductor comprised of a supporting substrate, a charge generating layer, a charge transport layer or charge transport layers, such as a first pass charge transport layer, and a second pass polysulfone containing charge transport layer, and which photoconductors possess a number of advantages, such excellent scratch and wear resistance; cyclic stability, deletion resistance, bias charging roll (BCR) wear resistance in xerographic imaging and printing systems; excellent photoconductor photosensitivities; an acceptable, and in embodiments a low  $V_c$ ; and minimization or prevention of  $V_c$  cycle up; compatibility with the photogenerating and charge transport resin binders; color print stability; and acceptable lateral charge migration (LCM) characteristics, such as for example, excellent LCM resistance.

Excellent cyclic stability of the photoconductor refers, for example, to almost no or minimal change in a generated known photoinduced discharge curve (PIDC), especially no or minimal residual potential cycle up after a number of charge/discharge cycles of the photoconductor, for example about 100 kilocycles, or xerographic prints of, for example, from about 80 to about 100 kiloprints. Excellent color print stability refers, for example, to substantially no or minimal change in solid area density, especially in 60 percent halftone prints, and no or minimal random color variability from print to print after a number of xerographic prints, for example 50 kiloprints.

Scratch and wear resistance of the photoconductors refer, for example, to almost no or minimal change in charge transport layer thickness or surface morphology after a number of xerographic prints, for example, 50 kiloprints.

Also disclosed are methods of imaging and printing, especially in xerographic systems, with the photoconductor

devices illustrated herein. These methods generally involve the formation of an electrostatic latent image on the imaging member, followed by developing the image with a toner composition comprised, for example, of thermoplastic resin, colorant, such as pigment, charge additive, and surface additive, reference U.S. Pat. Nos. 4,560,635; 4,298,697 and 4,338,390, the disclosures of which are totally incorporated herein by reference, subsequently transferring the image to a suitable substrate, and permanently affixing the image thereto. In those environments wherein the device is to be used in a printing mode, the imaging method involves the same operation with the exception that exposure can be accomplished with a laser device or image bar. More specifically, flexible belts disclosed herein can be selected for the Xerox Corporation iGEN3® machines that generate with some versions over 100 copies per minute. Processes of imaging, especially xerographic imaging and printing, including digital, and/or color printing, are thus encompassed by the present disclosure. The imaging members are, in embodiments, sensitive in the wavelength region of, for example, from about 400 to about 900 nanometers, and in particular from about 650 to about 850 nanometers, thus diode lasers can be selected as the light source. Moreover, the imaging members of this disclosure are useful in high resolution color xerographic applications, particularly high speed color copying and printing processes.

#### References

There is illustrated in U.S. Pat. No. 6,913,863, is a photoconductive imaging member comprised of a hole blocking layer, a photogenerating layer, and a charge transport layer, and wherein the hole blocking layer is comprised of a metal oxide; and a mixture of a phenolic compound and a phenolic resin wherein the phenolic compound contains at least two phenolic groups.

Further, in U.S. Pat. No. 4,555,463, there is illustrated a layered imaging member with a chloroindium phthalocyanine photogenerating layer. In U.S. Pat. No. 4,587,189, there is illustrated a layered imaging member with, for example, a perylene, pigment photogenerating component. Both of the aforementioned patents disclose an aryl amine component, such as N,N'-diphenyl-N,N'-bis(3-methylphenyl)-1,1'-biphenyl-4,4'-diamine dispersed in a polycarbonate binder as a hole transport layer. The above components, such as the photogenerating compounds and the aryl amine charge transport, can be selected for the imaging members of the present disclosure in embodiments thereof.

Illustrated in U.S. Pat. No. 5,521,306, the disclosure of which is totally incorporated herein by reference, is a process for the preparation of Type V hydroxygallium phthalocyanine comprising the in situ formation of an alkoxy-bridged gallium phthalocyanine dimer, hydrolyzing the dimer to hydroxygallium phthalocyanine, and subsequently converting the hydroxygallium phthalocyanine product to Type V hydroxygallium phthalocyanine.

Illustrated in U.S. Pat. No. 5,482,811, the disclosure of which is totally incorporated herein by reference, is a process for the preparation of hydroxygallium phthalocyanine photogenerating pigments which comprises hydrolyzing a gallium phthalocyanine precursor pigment by dissolving the hydroxygallium phthalocyanine in a strong acid, and then reprecipitating the resulting dissolved pigment in basic aqueous media; removing any ionic species formed by washing with water; concentrating the resulting aqueous slurry comprised of water and hydroxygallium phthalocyanine to a wet cake; removing water from said slurry by azeotropic distillation

with an organic solvent, and subjecting said resulting pigment slurry to mixing with the addition of a second solvent to cause the formation of said hydroxygallium phthalocyanine polymorphs.

Also, in U.S. Pat. No. 5,473,064, the disclosure of which is totally incorporated herein by reference, there is illustrated a process for the preparation of photogenerating pigments of hydroxygallium phthalocyanine Type V essentially free of chlorine, where a pigment precursor Type I chlorogallium phthalocyanine is prepared by the reaction of gallium chloride in a solvent, such as N-methylpyrrolidone, present in an amount of from about 10 to about 100 parts, with 1,3-diiminoisoindolene (DI<sup>3</sup>) in an amount of from about 1 to about 10 parts, for each part of gallium chloride that is reacted; hydrolyzing said pigment precursor chlorogallium phthalocyanine Type I by standard methods, for example acid pasting, whereby the pigment precursor is dissolved in concentrated sulfuric acid and then reprecipitated in a solvent, such as water, or a dilute ammonia solution, for example from about 10 to about 15 percent; and subsequently treating the resulting hydrolyzed pigment hydroxygallium phthalocyanine Type I with a solvent, such as N,N-dimethylformamide, present in an amount of from about 1 to about 50 volume parts, for each weight part of pigment hydroxygallium phthalocyanine that is used by, for example, ball milling the Type I hydroxygallium phthalocyanine pigment in the presence of spherical glass beads, approximately 1 to 5 millimeters in diameter, at room temperature, about 25° C., for a period of from about 12 hours to about 1 week, and preferably about 24 hours.

The appropriate components, and processes of the above recited patents may be selected for the present disclosure in embodiments thereof.

#### SUMMARY

Disclosed in embodiments are imaging members with many of the advantages illustrated herein, such as extended lifetimes of service of, for example, in excess of about 1,500, 40 000 imaging cycles; excellent electrical characteristics; stable electrical properties; excellent lateral charge migration (LCM) resistance; excellent deletion resistance; acceptable background and/or minimal charge deficient spots (CDS); consistent V<sub>r</sub> (residual potential) that is substantially flat or no change over a number of imaging cycles as illustrated by the generation of known PIDC (Photoinduced Discharge Curve), and the like. Also disclosed are layered photoresponsive imaging members which are responsive to near infrared radiation from about 700 to about 900 nanometers.

Further disclosed are layered flexible photoresponsive imaging members with sensitivity to visible light, and with mechanically robust charge transport layers.

Additionally disclosed are flexible imaging members with optional hole blocking layers comprised of metal oxides, phenolic resins, and optional phenolic compounds, and which phenolic compounds contain at least two, and more specifically, two to ten phenol groups or phenolic resins with, for example, a weight average molecular weight ranging from about 500 to about 3,000 permitting, for example, a hole blocking layer with excellent efficient electron transport which usually results in a desirable photoconductor low residual potential V<sub>low</sub>.

#### Embodiments

In aspects thereof, there is illustrated herein a photoconductor comprising a supporting substrate, a photogenerating

layer, and at least one charge transport layer, and wherein the at least one charge transport layer includes a polysulfone with a glass transition temperature of from about 250° C. to about 350° C.; a photoconductor comprising a supporting substrate, a photogenerating layer, and at least one charge transport layer comprised of at least one charge transport component and a polysulfone as represented by at least one of



and with a glass transition temperature of from about 250° C. to about 350° C., wherein aryl is one of



6  
-continued



and wherein x is from about 50 to about 90 weight percent, y is from about 10 to about 50 weight percent, and wherein the total thereof is about 100 percent; a photoconductor comprising a supporting substrate, a photogenerating layer, and a charge transport layer comprised of a charge transport component and a polysulfone as represented by



35 wherein x and y represent the number of repeating segments; an imaging member comprising an optional supporting substrate, a photogenerating layer, and at least one charge transport layer comprised of at least one charge transport component, and where the charge transport layer comprises a polysulfone; a photoconductor comprising a supporting substrate, a photogenerating layer, and a charge transport layer comprised of a charge, such as hole transport component, and a polysulfone component with a high  $T_g$ , or glass transition temperature of from about 250° C. to about 350° C., from about 275° C. to about 325° C., or from about 290° C. to about 315° C.; a photoconductor where the polysulfone is present in an amount of from about 0.1 to about 30 weight percent, from about 1 to about 20 weight percent, from 1 to about 10 weight percent, from 1 to about 5 weight percent, from about 4 to about 6 weight percent, and yet more specifically, about 2, 5, and 10 weight percent.

40 In embodiments thereof, there are disclosed polysulfone photoconductive members comprised of a supporting substrate, a photogenerating layer thereover, a polysulfone charge transport layer, and an overcoat charge transport layer; a photoconductive member with a photogenerating layer of a thickness of from about 0.1 to about 10 microns, and at least one polysulfone containing transport layer each of a thickness of from about 5 to about 100 microns; a xerographic imaging apparatus containing a charging component, a development component, a transfer component, and a fixing component, and wherein the apparatus contains a photoconductive imaging member comprised of a supporting substrate, and thereover a layer comprised of a photogenerating pigment and a polysulfone containing charge transport layer or layers, and thereover an overcoat charge transport layer, and where the transport layer is of a thickness of from about 10 to about 75 microns; a member wherein the polysulfone or mixtures thereof is present in an amount of from about 1 to about 20

weight percent, or from about 2 to about 10 weight percent; a member wherein the photogenerating layer contains a photogenerating pigment present in an amount of from about 10 to about 95 weight percent; a member wherein the thickness of the photogenerating layer is from about 0.2 to about 4 microns; a member wherein the photogenerating layer contains an inactive polymer binder; a member wherein the photogenerating binder is present in an amount of from about 20 to about 90 percent by weight, and wherein the total of all layer components is about 100 percent; a member wherein the photogenerating component is a hydroxygallium phthalocyanine or a titanyl phthalocyanine that absorbs light of a wavelength of from about 370 to about 950 nanometers; an imaging member wherein the supporting substrate is comprised of a conductive substrate comprised of a metal; an imaging member wherein the conductive substrate is aluminum, aluminized polyethylene terephthalate, or titanized polyethylene terephthalate; an imaging member wherein the photogenerating resinous binder is selected from the group consisting of known suitable polymers like polyesters, polyvinyl butyrals, polycarbonates, polystyrene-*b*-polyvinyl pyridine, and polyvinyl formals; an imaging member wherein the photogenerating pigment is a metal free phthalocyanine; a photoconductor wherein each of the charge transport layers, especially a first and second layer, comprises



wherein X is selected from the group consisting of at least one of alkyl, alkoxy, and halogen such as methyl and chloride; and in embodiments where there is a total of four X substituents on each of the four terminating rings; an imaging member wherein alkyl and alkoxy contain from about 1 to about 15 carbon atoms; an imaging member wherein alkyl contains from about 1 to about 5 carbon atoms; an imaging member wherein alkyl is methyl; a photoconductor wherein each of or at least one of the charge transport layers, especially a first and second charge transport layer, comprises



wherein X, Y and Z are independently selected from the group comprised of at least one of alkyl, alkoxy, aryl, and halogen, and in embodiments Z can be present, Y can be present, or both Y and Z are present; or wherein the charge transport component is



wherein X and Y are independently alkyl, alkoxy, aryl, a halogen, or mixtures thereof, an imaging member, and wherein, for example, alkyl and alkoxy contains from about 1 to about 15 carbon atoms; alkyl contains from about 1 to about 5 carbon atoms; and wherein the charge transport resinous binder is selected from the group consisting of polycarbonates, polyarylates, and polystyrene; a photoconductor for use in xerographic imaging and printing systems, such as the Xerox Corporation iGen3® machines, wherein the photogenerating pigment present in the photogenerating layer is comprised of chlorogallium phthalocyanine, titanyl phthalocyanine, or Type V hydroxygallium phthalocyanine prepared by hydrolyzing a gallium phthalocyanine precursor by dissolving the hydroxygallium phthalocyanine in a strong acid, and then reprecipitating the resulting dissolved precursor in a basic aqueous media; removing the ionic species formed by washing with water; concentrating the resulting aqueous slurry comprised of water and hydroxygallium phthalocyanine to a wet cake; removing water from the wet cake by drying; and subjecting the resulting dry pigment to mixing with the addition of a second solvent to cause the formation of the hydroxygallium phthalocyanine; an imaging member wherein the Type V hydroxygallium phthalocyanine has major peaks, as measured with an X-ray diffractometer, at Bragg angles (2 theta  $\pm 0.2^\circ$ ) 7.4, 9.8, 12.4, 16.2, 17.6, 18.4, 21.9, 23.9, 25.0, 28.1 degrees, and the highest peak at 7.4 degrees; a method of imaging wherein the imaging member is exposed to light of a wavelength of from about 400 to about 950 nanometers; a member wherein the photogenerating layer is situated between the substrate and the charge transport layer; a member wherein the charge transport layer is situated between the substrate and the photogenerating layer, and wherein the number of charge transport layers is two; a member wherein the photogenerating layer is of a thickness of from about 0.1 to about 25 microns; a member wherein the photogenerating component amount is from about 0.05 to about 20 weight percent, and wherein the photogenerating component is dispersed in from about 10 to about 80 weight percent of a polymer binder; a member wherein the thickness of the photogenerating layer is from about 0.1 to about 11 microns; a member wherein the photogenerating and charge transport layer components are contained in a polymer binder, and wherein the binder is present in an amount of from about 50 to about 90 percent by weight, and wherein the total of the layer components is about 100 percent; a photoconductor wherein the photogenerating resinous binder is selected from the group consisting of at least one of polyesters, polyvinyl butyrals, polycarbonates, polystyrene-*b*-polyvinyl pyridine, and polyvinyl formals; an imaging member wherein the photogenerating pigment is Type V hydroxygallium phthalocyanine, titanyl phthalocyanine, chlorogallium phthalocyanine, or mixtures thereof, and the charge transport layer contains a hole transport of N,N'-diphenyl-N,N'-bis(3-methylphenyl)-1,1'-biphenyl-4,4'-diamine, N,N'-bis(4-butylphenyl)-N,N'-di-p-tolyl-[p-terphenyl]-4,4'-diamine, N,N'-bis(4-butylphenyl)-N,N'-di-m-tolyl-[p-terphenyl]-4,4'-diamine,

9

N,N'-bis(4-butylphenyl)-N,N'-di-o-tolyl-[p-terphenyl]-4,4'-diamine, N,N'-bis(4-butylphenyl)-N,N'-bis-(4-isopropylphenyl)-p-[terphenyl]-4,4'-diamine, N,N'-bis(4-butylphenyl)-N,N'-bis -(2-ethyl-6-methylphenyl)-[p-terphenyl]-4,4'-diamine, N,N'-bis(4-butylphenyl)-N,N'-bis-(2,5-dimethylphenyl)-[p-terphenyl]-4,4'-diamine, N,N'-diphenyl-N,N'-bis(3-chlorophenyl)-[p-terphenyl]4,4'-diamine molecules, and wherein the hole transport resinous binder is selected from the group consisting of polycarbonates and polystyrene; an imaging member wherein the photogenerating layer contains a metal free phthalocyanine; an imaging member wherein the photogenerating layer contains an alkoxygallium phthalocyanine; a photoconductive imaging member with a blocking layer contained as a coating on a substrate, and an adhesive layer coated on the blocking layer; an imaging member further containing an adhesive layer and a hole blocking layer; a color method of imaging which comprises generating an electrostatic latent image on the imaging member, developing the latent image, transferring, and fixing the developed electrostatic image to a suitable substrate; polysulfone containing photoconductive imaging members comprised of a supporting substrate, a photogenerating layer, a hole transport layer, and a top overcoating layer in contact with the hole transport layer, or in embodiments in contact with the photogenerating layer, and in embodiments wherein a plurality of charge transport layers are selected, such as for example, from 2 to about 10, and more specifically, 2 may be selected; and a photoconductive imaging member comprised of an optional supporting substrate, a photogenerating layer, and a first, second, and third charge transport layer.

Examples of the polysulfones incorporated into the charge transport layer photoconductors disclosed herein are represented by at least one of



where aryl is, for example, at least one of



10

-continued



and where x and y represent the number of segments, and more specifically, where x is, for example, from about 50 to about 90 weight percent, or from about 60 to about 80 weight percent, and y is, for example, from about 10 to about 50 weight percent, or from about 20 to about 40 weight percent, and where the total of the percentages of x and y is about 100 percent; and which polysulfone possesses, in embodiments, a glass transition temperature of equal to or greater than about 50 250°C., and up to about 350°C.

The number average molecular weight of the polysulfone is, in embodiments, from about 10,000 to about 100,000, or from about 20,000 to about 50,000, and the weight average molecular weight of the polysulfone is from about 20,000 to 55 about 300,000, or from about 30,000 to about 100,000.

One specific example of a polysulfone selected for incorporation in the charge transport layer or layers is HTM 2600 obtained from HT Materials Inc., Albany, N.Y., which polysulfone possesses a number average molecular weight of 60 about 11,000, a weight average molecular weight of about 30,000, and a glass transition temperature of about 265°C.

## PHOTOCONDUCTOR LAYER EXAMPLES

65 There can be selected for the photoconductors disclosed herein a number of known layers, such as substrates, photo-generating layers, charge transport layers (CTL), hole block-

## 11

ing layers, adhesive layers, protective overcoat layers, and the like. Examples, thicknesses, specific components of many of these layers include the following.

The thickness of the substrate layer depends on many factors, including economical considerations, electrical characteristics, and the like, thus this layer may be of a substantial thickness, for example over 3,000 microns, such as from about 1,000 to about 3,500 microns, from about 1,000 to about 2,000 microns, from about 300 to about 700 microns, or of a minimum thickness of, for example, about 100 to about 500 microns. In embodiments, the thickness of this layer is from about 75 to about 300 microns, or from about 100 to about 150 microns.

The substrate may be opaque or substantially transparent, and may comprise any suitable material. Accordingly, the substrate may comprise a layer of an electrically nonconductive or conductive material, such as an inorganic or an organic composition. As electrically nonconducting materials, there may be employed various resins known for this purpose including polyesters, polycarbonates, polyamides, polyurethanes, and the like, which are flexible as thin webs. An electrically conducting substrate may be any suitable metal of, for example, aluminum, nickel, steel, copper, and the like, or a polymeric material, as described above, filled with an electrically conducting substance, such as carbon, metallic powder, and the like, or an organic electrically conducting material. The electrically insulating or conductive substrate may be in the form of an endless flexible belt, a web, a rigid cylinder, a sheet, and the like. The thickness of the substrate layer depends on numerous factors, including strength desired and economical considerations. For a drum, this layer may be of a substantial thickness of, for example, up to many centimeters, or of a minimum thickness of less than a millimeter. Similarly, a flexible belt may be of a substantial thickness of, for example, about 250 microns, or of a minimum thickness of less than about 50 microns, provided there are no adverse effects on the final electrophotographic device. In embodiments where the substrate layer is not conductive, the surface thereof may be rendered electrically conductive by an electrically conductive coating. The conductive coating may vary in thickness over substantially wide ranges depending upon the optical transparency, degree of flexibility desired, and economic factors.

Illustrative examples of substrates are as illustrated herein, and more specifically, layers selected for the imaging members of the present disclosure, and which substrates can be opaque or substantially transparent comprise a layer of insulating material including inorganic or organic polymeric materials, such as MYLAR® a commercially available polymer, MYLAR® containing titanium, a layer of an organic or inorganic material having a semiconductive surface layer, such as indium tin oxide or aluminum arranged thereon, or a conductive material inclusive of aluminum, chromium, nickel, brass, or the like. The substrate may be flexible, seamless, or rigid, and may have a number of many different configurations, such as for example, a plate, a cylindrical drum, a scroll, an endless flexible belt, and the like. In embodiments, the substrate is in the form of a seamless flexible belt. In some situations, it may be desirable to coat on the back of the substrate, particularly when the substrate is a flexible organic polymeric material, an anticurl layer, such as for example polycarbonate materials commercially available as MAKROLON®.

The photogenerating layer, in embodiments, is comprised of a number of known photogenerating pigments, such as for example, about 50 weight percent of Type V hydroxygallium phthalocyanine, titanyl phthalocyanine or chlorogallium

## 12

phthalocyanine, and about 50 weight percent of a resin binder like poly(vinyl chloride-co-vinyl acetate) copolymer, such as VMCH (available from Dow Chemical), or polycarbonate. Generally, the photogenerating layer can contain known photogenerating pigments, such as metal phthalocyanines, metal free phthalocyanines, alkylhydroxyl gallium phthalocyanines, hydroxygallium phthalocyanines, chlorogallium phthalocyanines, perylenes, especially bis(benzimidazo) perylene, titanyl phthalocyanines, and the like, and more specifically, vanadyl phthalocyanines, Type V hydroxygallium phthalocyanines, and inorganic components, such as selenium, selenium alloys, and trigonal selenium. The photogenerating pigment can be dispersed in a resin binder similar to the resin binders selected for the charge transport layer, or alternatively no resin binder need be present. Generally, the thickness of the photogenerating layer depends on a number of factors, including the thicknesses of the other layers, and the amount of photogenerating material contained in the photogenerating layer. Accordingly, this layer can be of a thickness of, for example, from about 0.05 to about 10 microns, and more specifically, from about 0.25 to about 2 microns when, for example, the photogenerating compositions are present in an amount of from about 30 to about 75 percent by volume. The maximum thickness of this layer, in embodiments, is dependent primarily upon factors, such as photosensitivity, electrical properties, and mechanical considerations. The photogenerating layer binder resin is present in various suitable amounts, for example from about 1 to about 50 weight percent, and more specifically, from about 1 to about 10 weight percent, and which resin may be selected from a number of known polymers, such as poly(vinyl butyral), poly(vinyl carbazole), polyesters, polycarbonates, polyarylates, poly(vinyl chloride), polyacrylates and methacrylates, copolymers of vinyl chloride and vinyl acetate, phenolic resins, polyurethanes, poly(vinyl alcohol), polyacrylonitrile, polystyrene, other known suitable binders, and the like. It is desirable to select a coating solvent that does not substantially disturb or adversely affect the previously coated layers of the device. Examples of coating solvents for the photogenerating layer are ketones, alcohols, aromatic hydrocarbons, halogenated aliphatic hydrocarbons, silanols, amines, amides, esters, and the like. Specific solvent examples are cyclohexanone, acetone, methyl ethyl ketone, methanol, ethanol, butanol, amyl alcohol, toluene, xylene, chlorobenzene, carbon tetrachloride, chloroform, methylene chloride, trichloroethylene, dichloroethane, tetrahydrofuran, dioxane, diethyl ether, dimethyl formamide, dimethyl acetamide, butyl acetate, ethyl acetate, methoxyethyl acetate, and the like.

The photogenerating layer may comprise amorphous films of selenium and alloys of selenium and arsenic, tellurium, germanium, and the like; hydrogenated amorphous silicon; and compounds of silicon and germanium, carbon, oxygen, nitrogen, and the like fabricated by vacuum evaporation or deposition. The photogenerating layers may also comprise inorganic pigments of crystalline selenium and its alloys; Groups II to VI compounds; and organic pigments, such as quinacridones, polycyclic pigments, such as dibromo anthranthrone pigments, perylene and perinone diamines, polynuclear aromatic quinones, azo pigments including bis-, tris- and tetrakis-azos; and the like dispersed in a film forming polymeric binder, and fabricated by solvent coating techniques.

Examples of binders for the photogenerating layer are thermoplastic and thermosetting resins, such as polycarbonates, polyesters, polyamides, polyurethanes, polystyrenes, polyarylsilanol, polyarylsulfones, polybutadienes, polysulfones,

polysilanolsulfones, polyethylenes, polypropylenes, polyimides, polymethylpentenes, poly(phenylene sulfides), poly(vinyl acetate), polysiloxanes, polyacrylates, polyvinyl acetals, polyamides, polyimides, amino resins, phenylene oxide resins, terephthalic acid resins, phenoxy resins, epoxy resins, phenolic resins, polystyrene and acrylonitrile copolymers, poly(vinyl chloride), vinyl chloride and vinyl acetate copolymers, acrylic copolymers, alkyd resins, cellulosic film formers, poly(amideimide), styrene butadiene copolymers, vinylidene chloride-vinyl chloride copolymers, vinyl acetate-vinylidene chloride copolymers, styrene-alkyd resins, poly(vinyl carbazole), and the like. These polymers may be block, random, or alternating copolymers.

The photogenerating composition or pigment is present in the resinous binder composition in various amounts. Generally, however, from about 5 to about 90 percent by weight of the photogenerating pigment is dispersed in about 10 to about 95 percent by weight of the resinous binder, or from about 20 to about 50 percent by weight of the photogenerating pigment is dispersed in about 80 to about 50 percent by weight of the resinous binder composition. In one embodiment, about 50 percent by weight of the photogenerating pigment is dispersed in about 50 percent by weight of the resinous binder composition.

Various suitable and conventional known processes may be used to mix, and thereafter apply the photogenerating layer coating mixture like spraying, dip coating, roll coating, wire wound rod coating, vacuum sublimation, and the like. For some applications, the photogenerating layer may be fabricated in a dot or line pattern. Removal of the solvent of a solvent-coated photogenerating layer may be effected by any known conventional techniques such as oven drying, infrared radiation drying, air drying, and the like.

The coating of the photogenerating layer in embodiments of the present disclosure can be accomplished to achieve a final dry thickness of the photogenerating layer as illustrated herein, and for example, from about 0.01 to about 30 microns after being dried at, for example, about 40° C. to about 150° C. for about 1 to about 90 minutes. More specifically, a photogenerating layer of a thickness, for example, of from about 0.1 to about 30 microns, or from about 0.5 to about 2 microns can be applied to or deposited on the substrate, on other surfaces in between the substrate and the charge transport layer, and the like. A charge blocking layer or hole blocking layer may optionally be applied to the electrically conductive surface prior to the application of a photogenerating layer. When desired, an adhesive layer may be included between the charge blocking, hole blocking layer, or interfacial layer, and the photogenerating layer. Usually, the photogenerating layer is applied onto the blocking layer, and a charge transport layer or plurality of charge transport layers are formed on the photogenerating layer. The photogenerating layer may be applied on top of or below the charge transport layer.

In embodiments, a suitable known adhesive layer can be included in the photoconductor. Typical adhesive layer materials include, for example, polyesters, polyurethanes, and the like. The adhesive layer thickness can vary, and in embodiments is, for example, from about 0.05 to about 0.3 micron. The adhesive layer can be deposited on the hole blocking layer by spraying, dip coating, roll coating, wire wound rod coating, gravure coating, Bird applicator coating, and the like. Drying of the deposited coating may be effected by, for example, oven drying, infrared radiation drying, air drying and the like.

An optional adhesive layer or layers usually in contact with or situated between the hole blocking layer and the

photogenerating layer, there can be selected various known substances inclusive of copolymers, polyamides, poly(vinyl butyral), poly(vinyl alcohol), polyurethane, and polyacrylonitrile. This layer is, for example, of a thickness of from about 0.001 to about 1 micron, or from about 0.1 to about 0.5 micron. Optionally, this layer may contain effective suitable amounts, for example from about 1 to about 10 weight percent, of conductive and nonconductive particles, such as zinc oxide, titanium dioxide, silicon nitride, carbon black, and the like, to provide, for example, in embodiments of the present disclosure further desirable electrical and optical properties.

The optional hole blocking or undercoat layer for the imaging members of the present disclosure can contain a number of components including known hole blocking components, such as amino silanes, doped metal oxides, a metal oxide like titanium, chromium, zinc, tin and the like; a mixture of phenolic compounds and a phenolic resin, or a mixture of two phenolic resins, and optionally a dopant such as SiO<sub>2</sub>. The phenolic compounds usually contain at least two phenol groups, such as bisphenol A (4,4'-isopropylidenediphenol), E (4,4'-ethylidenebisphenol), F (bis(4-hydroxyphenyl)methane), M (4,4'-(1,3-phenylenediisopropylidene)bisphenol), P (4,4'-(1,4-phenylene diisopropylidene)bisphenol), S (4,4'-sulfonyldiphenol), and Z (4,4'-cyclohexylidenebisphenol); hexafluorobisphenol A (4,4'-(hexafluoro isopropylidene) diphenol), resorcinol, hydroxyquinone, catechin, and the like.

The hole blocking layer can be, for example, comprised of from about 20 to about 80 weight percent, and more specifically, from about 55 to about 65 weight percent of a suitable component like a metal oxide, such as TiO<sub>2</sub>; from about 20 to about 70 weight percent, and more specifically, from about 25 to about 50 weight percent of a phenolic resin; from about 2 to about 20 weight percent, and more specifically, from about 5 to about 15 weight percent of a phenolic compound containing, for example, at least two phenolic groups, such as bisphenol S; and from about 2 to about 15 weight percent, and more specifically, from about 4 to about 10 weight percent of a plywood suppression dopant, such as SiO<sub>2</sub>. The hole blocking layer coating dispersion can, for example, be prepared as follows. The metal oxide/phenolic resin dispersion is first prepared by ball milling or dynamilling until the median particle size of the metal oxide in the dispersion is less than about 10 nanometers, for example from about 5 to about 9 nanometers. To the above dispersion are added a phenolic compound and dopant followed by mixing. The hole blocking layer coating dispersion can be applied by dip coating or web coating, and the layer can be thermally cured after coating. The hole blocking layer resulting is, for example, of a thickness of from about 0.01 to about 30 microns, and more specifically, from about 0.1 to about 8 microns. Examples of phenolic resins include formaldehyde polymers with phenol, p-tert-butylphenol, cresol, such as VARCUM® 29159 and 29101 (available from OxyChem Company), and DURITE® 97 (available from Borden Chemical); formaldehyde polymers with ammonia, cresol and phenol, such as VARCUM® 29112 (available from OxyChem Company); formaldehyde polymers with 4,4'-(1-methylethylidene)bisphenol, such as VARCUM® 29108 and 29116 (available from OxyChem Company); formaldehyde polymers with cresol and phenol, such as VARCUM® 29457 (available from OxyChem Company), DURITE® SD-423A, SD-422A (available from Borden Chemical); or formaldehyde polymers with phenol and p-tert-butylphenol, such as DURITE® ESD 556C (available from Borden Chemical).

In addition to the polysulfones, the charge transport layer includes a number of known materials as illustrated herein,

such as aryl amines, and which layer is generally of a thickness of from about 12 to about 75 microns, and more specifically, of a thickness of from about 12 to about 40 microns. Examples of charge transport layer components include



wherein X is alkyl, alkoxy, aryl, a halogen, or mixtures thereof, and especially those substituents selected from the group consisting of Cl and CH<sub>3</sub>; and molecules of the following formula



wherein X and Y are independently alkyl, alkoxy, aryl, a halogen, or mixtures thereof.

Alkyl and alkoxy contain, for example, from 1 to about 25 carbon atoms, and more specifically, from 1 to about 12 carbon atoms, such as methyl, ethyl, propyl, butyl, pentyl, and the corresponding alkoxides. Aryl can contain from 6 to about 36 carbon atoms, such as phenyl, and the like. Halogen includes chloride, bromide, iodide, and fluoride. Substituted alkyls, alkoxys, and aryls can also be selected in embodiments.

Examples of specific aryl amines include N,N'-diphenyl-N,N'-bis(alkylphenyl)-1,1-biphenyl-4,4'-diamine wherein alkyl is selected from the group consisting of methyl, ethyl, propyl, butyl, hexyl, and the like; N,N'-diphenyl-N,N'-bis(halophenyl)-1,1'-biphenyl-4,4'-diamine wherein the halo substituent is a chloro substituent; N,N'-bis(4-butylphenyl)-N,N'-di-p-tolyl-[p-terphenyl]-4,4'-diamine, N,N'-bis(4-butylphenyl)-N,N'-di-m-tolyl-[p-terphenyl]-4,4'-diamine, N,N'-bis(4-butylphenyl)-N,N'-di-o-tolyl-[p-terphenyl]-4,4'-diamine, N,N'-bis(4-butylphenyl)-N,N'-bis-(4-isopropylphenyl)-[p-terphenyl]-4,4'-diamine, N,N'-bis(4-butylphenyl)-N,N'-bis-(2-ethyl-6-methylphenyl)-[p-terphenyl]-4,4'-diamine, N,N'-bis(4-butylphenyl)-N,N'-bis-(2,5-dimethylphenyl)-[p-terphenyl]-4,4'-diamine, N,N'-diphenyl-N,N'-bis(3-chlorophenyl)-[p-terphenyl]-4,4'-diamine, and the like. Other known charge transport layer molecules can be selected, reference for example, U.S. Pat. Nos. 4,921,773; 4,464,450, the disclosures of which are totally incorporated herein by reference.

Examples of polymer binder materials for the charge transport layer or layers include polycarbonates, polyarylates, acrylate polymers, vinyl polymers, cellulose polymers, polyesters, polysiloxanes, polyamides, polyurethanes, poly(cycloolefins), epoxies, and random or alternating copolymers thereof; and more specifically, polycarbonates such as poly(4,4'-isopropylidene-diphenylene)carbonate (also referred to

as bisphenol-A-polycarbonate), poly(4,4'-cyclohexylidene diphenylene)carbonate (also referred to as bisphenol-Z-polycarbonate), poly(4,4'-isopropylidene-3,3'-dimethyl-diphenyl) carbonate (also referred to as bisphenol-C-polycarbonate), and the like. In embodiments, the charge transport layer binders are comprised of polycarbonate resins with a weight average molecular weight of from about 20,000 to about 100,000, or with a molecular weight M<sub>w</sub> of from about 50,000 to about 100,000 preferred. Generally, in embodiments the transport layer contains from about 10 to about 75 percent by weight of the charge transport material, and more specifically, from about 35 to about 50 percent of this material.

The charge transport layer or layers, and more specifically, a first charge transport in contact with the photogenerating layer, and thereover a top or second polysulfone charge transport overcoating layer may comprise charge transporting small molecules dissolved or molecularly dispersed in a film forming electrically inert polymer such as a polycarbonate. In embodiments, "dissolved" refers, for example, to forming a solution in which the small molecule and silanol are dissolved in the polymer to form a homogeneous phase; and "molecularly dispersed in embodiments" refers, for example, to charge transporting molecules dispersed in the polymer, the small molecules being dispersed in the polymer on a molecular scale. Various charge transporting or electrically active small molecules may be selected for the charge transport layer or layers. In embodiments, charge transport refers, for example, to charge transporting molecules as a monomer that allows the free charge generated in the photogenerating layer to be transported across the transport layer.

Examples of hole transporting molecules, especially for the first and second charge transport layers, and present, for example, in an amount of from about 45 to about 80 weight percent, include, for example, pyrazolines such as 1-phenyl-3-(4'-diethylamino styryl)-5-(4"-diethylamino phenyl)pyrazoline; aryl amines such as N,N'-diphenyl-N,N'-bis(3-methylphenyl)-(1,1'-biphenyl)-4,4'-diamine, N,N'-bis(4-butylphenyl)-N,N'-di-p-tolyl-[p-terphenyl]-4,4'-diamine, N,N'-bis(4-butylphenyl)-N,N'-di-m-tolyl-[p-terphenyl]-4,4'-diamine, N,N'-bis(4-butylphenyl)-N,N'-di-o-tolyl-[p-terphenyl]-4,4'-diamine, N,N'-bis(4-butylphenyl)-N,N'-bis(4-isopropylphenyl)-[p-terphenyl]-4,4'-diamine, N,N'-bis(4-butylphenyl)-N,N'-bis(2-ethyl-6-methylphenyl)-[p-terphenyl]-4,4'-diamine, N,N'-bis(4-butylphenyl)-N,N'-bis(2,5-dimethylphenyl)-[p-terphenyl]-4,4'-diamine, N,N'-diphenyl-N,N'-bis(3-chlorophenyl)-[p-terphenyl]-4,4'-diamine; hydrazones such as N-phenyl-N-methyl-3-(9-ethyl) carbazi hydrazone, and 4-diethyl amino benzaldehyde-1,2-diphenyl hydrazone; and a polysulfone.

The thickness of each of the charge transport layers, in embodiments, is from about 5 to about 75 microns, but thicknesses outside this range may, in embodiments, also be selected. The charge transport layer should be an insulator to the extent that an electrostatic charge placed on the hole transport layer is not conducted in the absence of illumination at a rate sufficient to prevent formation and retention of an electrostatic latent image thereon. In general, the ratio of the thickness of the charge transport layer to the photogenerating layer can be from about 2:1 to 200:1, and in some instances 400:1. The charge transport layer is substantially nonabsorbing to visible light or radiation in the region of intended use, but is electrically "active" in that it allows the injection of photogenerated holes from the photoconductive layer, or photogenerating layer, and allows these holes to be transported to selectively discharge a surface charge on the surface of the active layer.

The thickness of the continuous charge transport overcoat layer selected depends upon the abrasiveness of the charging (bias charging roll), cleaning (blade or web), development (brush), transfer (bias transfer roll), and the like in the system employed, and can be up to about 10 microns. In embodiments, this thickness for each layer is from about 1 to about 5 microns. Various suitable and conventional methods may be used to mix, and thereafter apply the overcoat layer coating mixture to the photoconductor. Typical application techniques include spraying, dip coating, roll coating, wire wound rod coating, and the like. Drying of the deposited coating may be effected by any suitable conventional technique, such as oven drying, infrared radiation drying, air drying, and the like. The dried overcoating layer of this disclosure should transport holes during imaging, and should not have too high a free carrier concentration.

The overcoat can comprise the same components as the charge transport layer wherein the weight ratio between the charge transporting small molecules, and the suitable electrically inactive resin binder is, for example, from about 0/100 to about 60/40, or from about 20/80 to about 40/60.

Examples of components or materials optionally incorporated into the charge transport layers or at least one charge transport layer to, for example, enable improved lateral charge migration (LCM) resistance include hindered phenolic antioxidants, such as tetrakis methylene(3,5-di-tert-butyl-4-hydroxy hydrocinnamate)methane (IRGANOX® 1010, available from Ciba Specialty Chemical), butylated hydroxytoluene (BHT), and other hindered phenolic antioxidants including SUMILIZER™ BHT-R, MDP-S, BBM-S, WX-R, NW, BP-76, BP-101, GA-80, GM and GS (available from Sumitomo Chemical Company, Ltd.), IRGANOX® 1035, 1076, 1098, 1135, 1141, 1222, 1330, 1425WL, 1520L, 245, 259, 3114, 3790, 5057 and 565 (available from Ciba Specialties Chemicals), and ADEKA STAB™ AO-20, AO-30, AO-40, AO-50, AO-60, AO-70, AO-80 and AO-330 (available from Asahi Denka Company, Ltd.); hindered amine antioxidants such as SANOL™ LS-2626, LS-765, LS-770 and LS-744 (available from SNKYCO CO., Ltd.), TINUVIN® 144 and 622LD (available from Ciba Specialties Chemicals), MARK™ LA57, LA67, LA62, LA68 and LA63 (available from Asahi Denka Co., Ltd.), and SUMILIZER™ PS (available from Sumitomo Chemical Co., Ltd.); thioether antioxidants such as SUMILIZER™ TP-D (available from Sumitomo Chemical Co., Ltd.); phosphite antioxidants such as MARK™ 2112, PEP-8, PEP-24G, PEP-36, 329K and HP-10 (available from Asahi Denka Co., Ltd.); other molecules, such as bis(4-diethylamino-2-methylphenyl)phenylmethane (BDETPM), bis-[2-methyl-4-(N-2-hydroxyethyl-N-ethyl-aminophenyl)]-phenylmethane (DHTPM), and the like. The weight percent of the antioxidant in at least one of the charge transport layers is from about 0 to about 20 weight percent, from about 1 to about 10 weight percent, or from about 3 to about 8 weight percent.

Primarily for purposes of brevity, the examples of each of the substituents, and each of the components/compounds/molecules, polymers, (components) for each of the layers, specifically disclosed herein are not intended to be exhaustive. Thus, a number of components, polymers, formulas, structures, and R group or substituent examples, and carbon chain lengths not specifically disclosed or claimed are intended to be encompassed by the present disclosure and claims. Also, the carbon chain lengths are intended to include all numbers between those disclosed or claimed or envisioned, thus from 1 to about 20 carbon atoms, and from 6 to about 36 carbon atoms includes 1, 2, 3, 4, 5, 6, 7, 8, 9, 10, 11, 12, 13, 14, 15, up to 36, or more. At least one refers, for

example, to from 1 to about 5, from 1 to about 2, 1, 2, and the like. Similarly, the thickness of each of the layers, the examples of components in each of the layers, the amount ranges of each of the components disclosed and claimed is not exhaustive, and it is intended that the present disclosure and claims encompass other suitable parameters not disclosed or that may be envisioned.

The following Examples are being submitted to illustrate embodiments of the present disclosure. These Examples are intended to be illustrative only, and are not intended to limit the scope of the present disclosure. Also, parts and percentages are by weight unless otherwise indicated. A Comparative Example and data are also provided.

15

#### Comparative Example 1

There was prepared a photoconductor with a biaxially oriented polyethylene naphthalate substrate (KALEDEX™ 2000) having a thickness of 3.5 mils, and thereover, a 0.02 micron thick titanium layer was coated on the biaxially oriented polyethylene naphthalate substrate (KALEDEX™ 2000). Subsequently, there was applied thereon, with an extrusion coater, a hole blocking layer solution containing 50 grams of 3 aminopropyl triethoxysilane ( $\gamma$ -APS), 41.2 grams of water, 15 grams of acetic acid, 684.8 grams of denatured alcohol, and 200 grams of heptane. This layer was then dried for about 1 minute at 120° C. in a forced air dryer. The resulting hole blocking layer had a dry thickness of 500 Angstroms. An adhesive layer was then deposited by applying a wet coating over the blocking layer, using an extrusion coater, and which adhesive contained 0.2 percent by weight based on the total weight of the solution of the copolyester adhesive (ARDEL D100™ available from Toyota Hsutsu Inc.) in a 60:30:10 volume ratio mixture of tetrahydrofuran/monochlorobenzene/methylene chloride. The adhesive layer was then dried for about 1 minute at 120° C. in the forced air dryer of the coater. The resulting adhesive layer had a dry thickness of 200 Angstroms.

A photogenerating layer dispersion was prepared by introducing 0.45 gram of the known polycarbonate IUPILON 200™ (PCZ-200) weight average molecular weight of 20,000, available from Mitsubishi Gas Chemical Corporation, and 44.65 grams of tetrahydrofuran (THF) into a 4 ounce glass bottle. To this solution were added 2.4 grams of hydroxygallium phthalocyanine (Type V) and 300 grams of  $\frac{1}{8}$  inch (3.2 millimeters) diameter stainless steel shot. This mixture was then placed on a ball mill for 3 hours. Subsequently, 2.25 grams of PCZ-200 were dissolved in 46.1 grams of THF, and added to the hydroxygallium phthalocyanine dispersion. This slurry was then placed on a shaker for 10 minutes. The resulting dispersion was, thereafter, applied to the above adhesive interface with an extrusion coater. A strip about 10 millimeters wide along one edge of the substrate web bearing the blocking layer and the adhesive layer was deliberately left uncoated by any of the photogenerating layer material to facilitate adequate electrical contact by a known ground strip layer that was applied later. The photogenerating layer was dried at 120° C. for 1 minute in a forced air oven to form a dry photogenerating layer of hydroxygallium phthalocyanine Type V and PCZ-200 with a weight ratio of about 47/53, and having a thickness of 0.8 micron.

The resulting imaging member web was then overcoated with two charge transport layers. Specifically, the photogenerating layer was overcoated with a first pass charge transport layer (the bottom layer) in contact with the photogenerating layer. The bottom layer of the charge transport layer was prepared by introducing into an amber glass bottle in a weight

19

ratio of 50/50 N,N'-diphenyl-N,N'-bis(3-methylphenyl)-1,1'-biphenyl-4,4'-diamine (mTBD) and MAKROLON® 5705, a known polycarbonate resin having a molecular weight average of from about 50,000 to about 100,000, commercially available from Farbenfabriken Bayer A.G. The resulting mixture was then dissolved in methylene chloride to form a solution containing 15 percent by weight solids. This solution was applied on the photogenerating layer to form the bottom layer coating that upon drying (120° C. for 1 minute) had a thickness of 14.5 microns. During this coating process, the humidity was equal to or somewhat less than 15 percent, such as from 12 to 15 percent.

The above bottom layer of the charge transport layer was then overcoated with a second pass top layer. The charge transport layer solution of the top layer was prepared by introducing into an amber glass bottle in a weight ratio of 35:65 N,N'-diphenyl-N,N'-bis(3-methylphenyl)-1,1'-biphenyl-4,4'-diamine (mTBD) and MAKROLON® 5705, a known polycarbonate resin having a molecular weight average of from about 50,000 to about 100,000, commercially available from Farbenfabriken Bayer A.G. The resulting mixture was then dissolved in methylene chloride to form a solution containing 15 percent by weight solids. The resulting top layer solution was applied on the bottom layer of the charge transport layer to form a coating that upon drying (120° C. for 1 minute) had a thickness of 14.5 microns. During this coating process, the humidity was equal to or somewhat less than 15 percent, such as from 12 to 15 percent.

#### Comparative Example 2

On a 30 millimeter aluminum drum substrate, an undercoat layer was prepared and deposited thereon as follows. Zirconium acetylacetone tributoxide (35.5 parts),  $\gamma$ -aminopropyl triethoxysilane (4.8 parts), and poly(vinyl butyral) BM-S (2.5 parts) were dissolved in n-butanol (52.2 parts). The resulting solution was then coated by a dip coater on the above aluminum drum substrate, and the coating solution layer was pre-heated at 59° C. for 13 minutes, humidified at 58° C. (dew point=54° C.) for 17 minutes, and dried at 135° C. for 8 minutes. The thickness of the undercoat layer was approximately 1.3 microns.

A photogenerating layer comprising chlorogallium phthalocyanine (Type C) was deposited on the above undercoat layer at a thickness of about 0.2 micron. The photogenerating layer coating dispersion was prepared as follows. 2.7 Grams of chlorogallium phthalocyanine (ClGaPc) Type C pigment were mixed with 2.3 grams of the polymeric binder (carboxyl-modified vinyl copolymer, VMCH, Dow Chemical Company), 15 grams of n-butyl acetate, and 30 grams of xylene. The resulting mixture was milled in an Attritor mill with about 200 grams of 1 millimeter Hi-Bea borosilicate glass beads for about 3 hours. The dispersion mixture obtained was then filtered through a 20  $\mu$ m Nylon cloth filter, and the solids content of the dispersion was diluted to about 6 weight percent.

Subsequently, a 32 thick micron charge transport layer was coated on top of the photogenerating layer from a solution prepared by dissolving N,N'-diphenyl-N,N'-bis(3-methylphenyl)-1,1'-biphenyl-4,4'-diamine (mTBD, 4 grams), and a film forming polymer binder PCZ-400 [poly(4,4'-dihydroxy-diphenyl-1-1-cyclohexane,  $M_w$ =40,000)] available from Mitsubishi Gas Chemical Company, Ltd. (6 grams) in a solvent mixture of 21 grams of tetrahydrofuran (THF) and 9 grams of toluene. The charge transport layer of PCZ-400/mTBD ratio was 60/40, and was dried at about 120° C. for about 40 minutes.

#### Example I

Three photoconductive members were prepared by repeating the process of Comparative Example 1 except that there

20

was included in the second pass or top charge transport layer 2, 4.8, and 9.1 weight percent of the polysulfone, HTM 2600 as obtained from HT Materials Inc., Albany, N.Y., which polysulfone possesses a number average molecular weight of about 11,000, a weight average molecular weight of about 30,000, and a glass transition temperature of about 265° C.

The resulting second pass or top charge transport layer solution was applied on the bottom or first pass charge transport layer to form a coating that upon drying (120° C. for 1 minute) had a thickness of 14.5 microns, where the weight 10 ratio of mTBD/MAKROLON® 5705/polysulfone in each of the second pass charge transport layers was 34.3/63.7/2 (A), 33.3/61.9/4.8 (B), and 31.8/59.1/9.1 (C). During this coating process, the humidity was equal to or somewhat less than 15 percent, such as from 12 to 15 percent.

15

#### Example II

A photoconductive member was prepared by repeating the process of Comparative Example 2 except that the charge transport layer solution was prepared by dissolving N,N'-diphenyl-N,N'-bis(3-methylphenyl)-1,1'-biphenyl-4,4'-diamine (mTBD, 4 grams), a film forming polymer binder PCZ-400 [poly(4,4'-dihydroxy-diphenyl-1-1-cyclohexane,  $M_w$ =40,000)] available from Mitsubishi Gas Chemical Company, Ltd. (6 grams), and the polysulfone, HTM 2600 as obtained from HT Materials Inc., Albany, N.Y., which polysulfone possessed a number average molecular weight of about 11,000, a weight average molecular weight of about 30,000, and a glass transition temperature of about 265° C. (0.5 gram) in a solvent mixture of 21 grams of tetrahydrofuran (THF) and 9 grams of toluene. The charge transport layer of PCZ-400/mTBD/polysulfone ratio was 57.1/38.1/4.8, and was dried at about 120° C. for about 40 minutes.

#### Electrical Property Testing

35 The above prepared photoconductor devices of Comparative Example 1 and Examples I (A), I (B), I (C), Comparative Example 2 and Example II were tested in a scanner set to obtain photoinduced discharge cycles, sequenced at one charge-erase cycle followed by one charge-expose-erase 40 cycle, wherein the light intensity was incrementally increased with cycling to produce a series of photoinduced discharge characteristic curves from which the photosensitivity and surface potentials at various exposure intensities are measured. Additional electrical characteristics were obtained by a series of charge-erase cycles with incrementing surface potential to generate several voltage versus charge density 45 curves. The scanner was equipped with a scorotron set to a constant voltage charging at various surface potentials. The devices were tested at surface potentials of 500 volts with the exposure light intensity incrementally increased by means of 50 regulating a series of neutral density filters; the exposure light source was a 780 nanometer light emitting diode. Xerographic simulation was completed in an environmentally controlled light tight chamber at ambient conditions (40 percent relative humidity and 22° C.).

55 Similar PIDC curves were obtained for the above photoconductors of Comparative Example 1 and Examples I (A), I (B), I (C), and Comparative Example 2, and Example II, respectively. Thus, incorporation of the polysulfone into the charge transport layer had substantially no negative impact on the electrical properties of the photoconductors when the photoconductors were in a belt photoconductor form or a drum photoconductor form.

#### Scratch Resistance Testing

65 Samples of the Comparative Example 1 and the Examples I (B) and I (C) belt photoconductors were cut into strips of 1

21

inch in width by 12 inches in length and were flexed in a tri-roller flexing system. Each belt was under a 1.1 lb/inch tension and each roller was  $\frac{1}{8}$  inches in diameter. A polyurethane "spots blade" was placed in contact with each belt at an angle between 5 and 15 degrees. Carrier beads of about 100 microns in size diameter were attached to the spots blade by the aid of double tape. The above photoconductive belts were flexed for 200 cycles in a in-house flexing fixture. The surface morphology of each scratched area was then analyzed.  $R_q$ , the root mean square roughness, was selected to be the standard metric for scratch resistance assessment. The results are provided in the following Table 1.

TABLE 1

| Photoconductors                                                                                    | $R_q$ (micron) |
|----------------------------------------------------------------------------------------------------|----------------|
| Comparative Example 1                                                                              | 0.230          |
| Example I (B) with 4.8 Weight Percent of the Polysulfone in the Second Pass Charge Transport Layer | 0.098          |
| Example I (C) with 9.1 Weight Percent of the Polysulfone in the Second Pass Charge Transport Layer | 0.137          |

Incorporation of the polysulfone into the charge transport layer reduced  $R_q$ , which indicated that the disclosed belt photoconductors were more scratch resistant than the Comparative Example 1 photoconductor. More specifically, incorporation of 4.8 weight percent of the polysulfone into the charge transport layer reduced the  $R_q$  by about 60 percent, and incorporation of 9.1 weight percent of the polysulfone into the charge transport layer reduced the  $R_q$  by about 40 percent as compared to that of the Comparative Example 1 belt photoconductor.

#### Wear Testing

Wear tests of the above Comparative Example 2 and Example II photoconductors were performed using a FX469 (Fuji Xerox) wear fixture. The total thickness of each photoconductor was measured via Permascope before each wear test was initiated. Then the photoconductors were separately placed into the wear fixture for 50 kcycles. The total thickness was measured again, and the difference in thickness was used to calculate wear rate (nanometers/kilocycle) of the photoconductor. The smaller the wear rate number, the more wear resistant is the photoconductor. The wear rate data is summarized in Table 2.

TABLE 2

|                                                                                     | WEAR RATE<br>(nanometers/<br>kilocycle) |
|-------------------------------------------------------------------------------------|-----------------------------------------|
| Comparative Example 2                                                               | 60                                      |
| Example II with 4.8 Weight Percent of the Polysulfone in the Charge Transport Layer | 40                                      |

For a bias charging roll xerographic system, the drum photoconductor of Example II exhibited significantly more wear resistance (about 35 percent) than the controlled photoconductor of Comparative Example 2, thus incorporation of the polysulfone into the charge transport layer improved the wear resistance of the photoconductor.

The claims, as originally presented and as they may be amended, encompass variations, alternatives, modifications, improvements, equivalents, and substantial equivalents of the embodiments and teachings disclosed herein, including those that are presently unforeseen or unappreciated, and that, for

22

example, may arise from applicants/patentees and others. Unless specifically recited in a claim, steps or components of claims should not be implied or imported from the specification or any other claims as to any particular order, number, position, size, shape, angle, color, or material.

What is claimed is:

1. A photoconductor consisting of a supporting substrate, a photogenerating layer, an optional hole blocking layer, an optional adhesive layer, and at least one charge transport layer, and wherein said at least one charge transport layer includes a polysulfone with a glass transition temperature of from about 250° C. to about 350° C., and an optional antioxidant, wherein said polysulfone is represented by



wherein x is from about 60 to about 80, y is from about 20 to about 40, and wherein the total thereof is about 100, and wherein aryl is at least one of



23

-continued



2. A photoconductor in accordance with claim 1 wherein said polysulfone is represented by



3. A photoconductor in accordance with claim 1 wherein said polysulfone is present in said at least one charge transport layer in an amount of from about 0.1 to about 30 weight percent of the total solids.

4. A photoconductor in accordance with claim 1 wherein said polysulfone is present in said at least one charge transport layer in an amount of from about 1 to about 20 weight percent of the total solids, and wherein at least one charge transport layer is 1 layer, 2 layers, or 3 layers.

5. A photoconductor in accordance with claim 1 wherein said polysulfone possesses a glass transition temperature of from about 250° C. to about 300° C.

6. A photoconductor in accordance with claim 1 wherein said polysulfone possesses a weight average molecular weight of from about 20,000 to about 300,000, and at least one charge transport layer is 1, or 2 layers.

7. A photoconductor in accordance with claim 1 wherein said polysulfone possesses a weight average molecular weight of from about 30,000 to about 100,000.

8. A photoconductor in accordance with claim 1 wherein said charge transport layer consists of said polysulfone, and a charge transport component as represented by

24



wherein X is selected from the group consisting of alkyl, alkoxy, aryl, and halogen, and mixtures thereof, and wherein at least one charge transport layer is from 1 to about 3 layers.

9. A photoconductor in accordance with claim 8 wherein said alkyl and said alkoxy each contains from about 1 to about 12 carbon atoms, and said aryl contains from about 6 to about 36 carbon atoms; and wherein said polysulfone is present in an amount of from about 1 to about 10 weight percent of the total solids.

10. A photoconductor in accordance with claim 8 wherein said charge transport component is N,N'-diphenyl-N,N-bis(3-methylphenyl)-1,1'-biphenyl-4,4'-diamine.

11. A photoconductor in accordance with claim 1 wherein said charge transport layer consists of said polysulfone, and said charge transport layer contains a hole transport component as represented by



40 wherein X, Y, and Z are independently selected from the group consisting of alkyl, alkoxy, aryl, and halogen, and mixtures thereof.

12. A photoconductor in accordance with claim 1 wherein said charge transport layer includes a component selected

45 from at least one of the group consisting of N,N'-bis(4-butylphenyl)-N,N'-di-p-tolyl-[p-terphenyl]-4,4'-diamine, N,N'-bis(4-butylphenyl)-N,N'-di-m-tolyl-[p-terphenyl]-4,4'-diamine, N,N'-bis(4-butylphenyl)-N,N'-di-o-tolyl-[p-terphenyl]-4,4'-diamine, N,N'-bis(4-butylphenyl)-N,N'-bis(4-isopropylphenyl)-[p-terphenyl]-4,4'-diamine, N,N'-bis(4-butylphenyl)-N,N'-bis(2-ethyl-6-methylphenyl)-[p-terphenyl]-4,4'-diamine, N,N'-bis(4-butylphenyl)-N,N'-bis(2,5-dimethylphenyl)-[p-terphenyl]-4,4'-diamine, N,N'-diphenyl-N,N-bis(3-methylphenyl)-1,1'-biphenyl-4,4'-diamine, and N,N'-diphenyl-N,N'-bis(3-chlorophenyl)-[p-terphenyl]-4,4'-diamine; and wherein said at least one charge transport layer is 1, 2, or 3 layers, and said polysulfone is present in an amount of from about 1 to about 10 weight percent of the total solids.

13. A photoconductor in accordance with claim 1 wherein said antioxidant is present and consists of a hindered phenolic, a hindered amine, or mixtures thereof.

14. A photoconductor in accordance with claim 1 wherein said photogenerating layer consists of a photogenerating pigment or photogenerating pigments and an optional binder.

15. A photoconductor in accordance with claim 14 wherein said photogenerating pigment consists of at least one of a

25

titanyl phthalocyanine, a hydroxygallium phthalocyanine, a halogallium phthalocyanine, a perylene, or mixtures thereof, and said at least one charge transport layer is 1, 2, or 3 layers.

**16.** A photoconductor in accordance with claim 14 wherein said photogenerating pigment consists of a metal phthalocyanine, a metal free phthalocyanine, or mixtures thereof.

**17.** A photoconductor in accordance with claim 14 wherein said photogenerating pigment is a hydroxygallium phthalocyanine.

**18.** A photoconductor in accordance with claim 1 wherein said hole blocking layer, and said adhesive layer are present, and wherein said polysulfone is present in an amount of from about 2 to about 10 weight percent of the total solids.

**19.** A photoconductor in accordance with claim 1 wherein said at least one charge transport layer is from 1 to about 4 layers.

20. A photoconductor in accordance with claim 1 wherein  
said at least one charge transport layer consists of a top charge  
transport layer and a bottom charge transport layer, and  
wherein said top charge transport layer is in contact with said  
bottom charge transport layer and said bottom charge trans-  
port layer is in contact with said photogenerating layer, and  
wherein said polysulfone is present in said top charge trans-  
port layer in an amount of from about 1 to about 10 weight  
percent of the total solids.

**21.** A photoconductor in accordance with claim 1 wherein said polysulfone is



wherein at least one charge transport layer is 1, 2, or 3 layers.

22. A photoconductor in accordance with claim 21 wherein said polysulfone is present in an amount of about 2, about 5, 40 or about 9 weight percent of the total solids.

23. A photoconductor in accordance with claim 1 wherein said polysulfone is present in an amount of about 2, about 5, or about 9 weight percent of the total solids.

**24.** A photoconductor consisting of a supporting substrate, 45 a photogenerating layer, and at least one charge transport layer consisting of at least one charge transport component and a polysulfone as represented by at least one of



and with a glass transition temperature of from about 250° C. to about 350° C., wherein aryl is one of

26



50 and wherein x is 60 to 80, y is 20 to 40, and wherein the total thereof is about 100, and wherein said charge transport component is represented by the following structures/formulas



wherein X, Y, and Z are independently selected from the group consisting of alkyl, alkoxy, aryl, and halogen.

**27**

25. A photoconductor in accordance with claim 24 wherein at least one charge transport layer is two layers, a first charge transport layer in contact with the photogenerating layer and a second charge transport layer in contact with the first charge transport layer, wherein said polysulfone is present in said second charge transport layer in an amount of from about 1 to about 10 weight percent of the total solids, and wherein said polysulfone possesses a glass transition temperature of from about 250° C. to about 310° C.

26. A photoconductor consisting of a supporting substrate, a photogenerating layer, and a charge transport layer consisting of a mixture of a charge transport component and a polysulfone as represented by

**28**

wherein x is from about 60 to about 80, y is from about 20 to about 40, and wherein the total thereof is about 100, wherein said polysulfone has a number average molecular weight of from about 20,000 to about 50,000, and a weight average molecular weight of about 30,000 to about 100,000, and wherein said polysulfone possesses a glass transition temperature of about 290° C. to about 310° C.

10 27. A photoconductor in accordance with claim 26 wherein said polysulfone is present in an amount of from 1 to about 12 weight percent of the total solids; and wherein aryl contains from 6 to about 36 carbon atoms.

15 28. A photoconductor in accordance with claim 26 wherein said polysulfone is present in an amount of about 2, about 5, or about 9 weight percent of the total solids.

\* \* \* \* \*